

## UNITED STATES PATENT OFFICE.

MARION B. HOPKINS, OF ELIZABETH, AND HYYM E. BUC, OF ROSELLE, NEW JERSEY,  
ASSIGNORS TO STANDARD OIL DEVELOPMENT COMPANY, A CORPORATION OF  
DELAWARE.

## CELLULOSE-NITRATE SOLUTION.

No Drawing.

Application filed April 3, 1922. Serial No. 549,189.

In a co-pending application of one of us, Serial No. 544,949, filed March 18, 1922, the preparation of nitro-compounds of non-benzenoid hydrocarbons has been described, the 5 resulting nitro-compounds consisting apparently chiefly of mono and di-nitro derivatives. The crude mixture of nitro-compounds may be separated by steam distillation into a mixture consisting largely of mono-nitro 10 pounds on the one hand and a mixture consisting largely of di-nitro compounds on the other hand. The nitro-compounds described in the above-mentioned application may be derived from liquid hydrocarbons or mixtures 15 thereof, for example, from gasoline or from close-cuts made by the fractional distillation of gasoline, or from individual hydrocarbons, for example, the range of hydrocarbons having from 6 to 12 carbon atoms, 20 or higher.

In accordance with the present invention, solutions of cellulose nitrate are prepared, employing mixtures of the mono or di-nitro compounds or both above referred to, together with alcohol as a primary solvent. The 25 alcohols used in such admixtures have been, for example, methyl alcohol, ethyl alcohol (95%), absolute ethyl alcohol, isopropyl alcohol, normal or secondary butyl alcohol, 30 amyl alcohol and the like. Benzol may be admixed with the resulting solution in very considerable proportions without causing precipitation of the cellulose nitrate. Other cellulose nitrate solvents may be added; for example, ethyl acetate, acetone, butyl acetate, 35 amyl acetate, or the like.

The proportion of solvent or solvents employed may be varied within wide limits, in accordance with the desired viscosity of the 40 resulting solution. The following examples illustrate solutions made in accordance with the present invention:

*Example No. 1.*

45 100 grams cellulose nitrate are dissolved in a mixture of 150 cubic centimeters of mono-nitro compounds and 400 cubic centimeters of ethyl alcohol (95%). A clear solution results, to which up to 300 cubic centimeters of benzol may be added without precipitation of the cellulose nitrate. Any less proportion of benzol may, of course, be employed if desired.

In the above example, absolute ethyl alcohol or other alcohols, for example, those above

mentioned, may be substituted for the 95% 55 ethyl alcohol. The same is true in the formulas hereinafter set forth in which the use of 95% alcohol is described. In the above example, the mono-nitro compounds employed are the steam volatile products of nitration, consisting largely of mono-nitro compounds. The mono-nitro compounds employed successfully in the above formula have been those derived from various cuts from gasoline, for example, the cut between 150 60 and 175° C., and likewise those derived from separated hydrocarbons, such as octane, nonane, etc.

*Example No. 2.*

70 200 grams of cellulose nitrate are dissolved in a mixture of 400 cubic centimeters of di-nitro compounds and 900 cubic centimeters of 75 95% ethyl alcohol. Any proportion of benzol up to 1500 cubic centimeters could be added to the resulting solution without precipitation of the cellulose nitrate.

The di-nitro compounds referred to above are the nitro-compounds not volatile with steam formed by nitration of hydrocarbons, for example, by the process referred to. They consist largely, but not entirely, of di-nitro compounds. The di-nitro products derived from the hydrocarbons of octane, nonane, or from any suitable gasoline fractions, may, for 80 85 example, be employed in the formula of this example.

In either of the above examples, the mixed 90 nitro-compounds produced in accordance with the process of the application hereinbefore referred to may be employed instead of the mono or di-nitro compounds specifically mentioned.

The following additional examples illustrate the use of the mixture of nitro-compounds and alcohol with other solvents and produce solutions having desirable properties.

*Example No. 3.*

100 100 grams of cellulose nitrate were dissolved in 750 cubic centimeters of mono-nitro products, 75 cubic centimeters mixed nitro products, 150 cubic centimeters 95% ethyl alcohol and 75 cubic centimeters ethyl acetate. 105 500 cubic centimeters of benzol were added to the solution, a clear liquid resulting.

In a modification of the above formula, the benzol was omitted and a total quantity

of 225 cubic centimeters of 95% ethyl alcohol were employed. Other solvents, such as butyl acetate, amyl acetate, or acetone, may be substituted for the ethyl acetate.

5 *Example No. 4.*

200 grams of cellulose nitrate were dissolved in 350 cubic centimeters of mixed nitro products, 500 cubic centimeters of 95% 10 ethyl alcohol and 100 cubic centimeters of acetone. 700 cubic centimeters of benzol were added without precipitating cellulose nitrate from the solution.

The mixed nitro products referred to in the 15 examples 3 and 4 are the mixtures of mono and di-nitro compounds formed by nitration of gasoline fractions such as those boiling between 150 and 175° C. The nitro-compounds derived from aliphatic hydrocarbons, such as 20 hexane, octane, nonane, or other hydrocarbons, may be substituted therefor.

We claim:

1. A solution of cellulose nitrate in a mixture of nitro-compounds of non-benzenoid 25 hydrocarbons and an alcohol.
2. A solution of cellulose nitrate in a mixture containing nitro-compounds of non-benzenoid hydrocarbons lower than trinitro derivatives and an alcohol.
- 30 3. A solution of cellulose nitrate in a mix-

ture of nitro-compounds of non-benzenoid hydrocarbons, an alcohol, and benzol.

4. A solution of cellulose nitrate in a mixture containing nitro-compounds of aliphatic hydrocarbons and ethyl alcohol.

35 5. A solution of cellulose nitrate in a liquid mixture containing nitro-compounds of aliphatic hydrocarbons, ethyl alcohol and benzol.

6. A solution of cellulose nitrate in a liquid 40 mixture containing nitro-compounds of paraffine hydrocarbons and 95% ethyl alcohol.

7. A solution of cellulose nitrate in a liquid 45 mixture containing nitro-compounds of paraffine hydrocarbons lower than trinitro compounds, 95% ethyl alcohol and benzol.

8. A solution of cellulose nitrate in a liquid mixture containing nitro-compounds of paraffine hydrocarbons lower than trinitro compounds, 95% ethyl alcohol and an added cellulose nitrate solvent.

9. A solution of cellulose nitrate in a mixture of nitro-compounds of aliphatic hydrocarbons, an alcohol and benzol.

10. A solution of cellulose nitrate in a mixture 55 of nitro-compounds of aliphatic hydrocarbons, an alcohol and an added cellulose nitrate solvent.

MARION B. HOPKINS.  
HYM E. BUC.